# EUROPEAN PATENT SPECIFICATION

(11) **EP 3 817 860 B1**
(45) Date of publication and mention of the grant of the patent: **04.09.2024**
(21) Application number: 19734426.0
(22) Date of filing: 04.07.2019
(51) Int. Cl.: B03D 1/008, B03D 1/004, B03D 1/01, B03D 1/02

(54) **PROCESS FOR FROTH FLOTATION**
SCHAUMFLOTATIONSVERFAHREN
PROCÉDÉ DE FLOTTATION PAR MOUSSE

(30) Priority: 06.07.2018 EP 18182117
(43) Date of publication of application: 12.05.2021
(73) Proprietor: Nouryon Chemicals International B.V., 6824 BM Arnhem (NL)
(72) Inventor: NORDBERG, Henrik, 444 53 Stenungsund (SE); GOLETS, Mikhail, 444 85 Stenungsund (SE); KLEBERGER HELLSTRÖM, Åsa Hele'n Jeanette, 459 33 Ljungskile (SE); DE LIMA, Odair Alves, 05579-000 São Paulo (BR); ALBINO, Kelly Ivone Pina, 13221-560 São Paulo (BR)
(74) Representative: LKGlobal UK Ltd.
(86) International application number: PCT/EP2019/067975
(87) International publication number: WO 2020/007971

(56) References cited:
- DE-A1- 4 016 792
- RU-C1- 2 288 040
- US-A- 5 443 158
- US-A1- 2017 252 753

## Description

### BACKGROUND

Phosphate rocks contain calcium phosphate minerals largely in the form of apatite, usually together with other minerals (*e*.*g*., silicate minerals and carbonate minerals, such as calcite). Apatite is a generic name for a group of calcium phosphate minerals also containing other elements or radicals, such as fluorapatite, chlorapatite, hydroxylapatite, carbonate-rich fluorapatite and carbonate-rich hydroxylapatite.

It is well-known to separate the valuable phosphate minerals from the gangue (commercially unimportant material) by using a froth flotation process where the phosphate minerals are enriched in the float. Good performance in a froth flotation process is achieved by a combination of, on the one hand, a good separation of the valuable mineral from the gangue by using a selective collector composition and, on the other hand, the froth characteristics, if needed by using frothers during the process which are then added in a step after the pulped ore has been conditioned with the collector composition. The froth characteristics include both the volume (height) and the stability of the froth. It is important in the flotation process that the froth collapses as soon as possible after the air supply is stopped, since this is directly connected to the flotation performance. A too stable froth will cause both entrainment of particles and froth product pumping problems. Entrainment, especially on a large scale, will result in decreased selectivity (i.e. grade, recovery). Problems with froth product pumping will make a flotation process technically impossible.

Collector performance may be improved by using collector combinations of a primary (main) collector and a secondary collector (also called co-collector). In this document the term "collector composition" shall be used to describe compositions containing a primary collector, or both a primary and a secondary collector, as well as a collector aid. For many decades secondary collectors have been used together with primary ionic collectors in salt-type mineral flotation to improve the performance of the primary collector. Nonylphenol ethoxylates have been the dominating nonionic surfactant used as a co-collector in a combination with sarcosine-type primary collectors in selective flotation of apatite from calcite-containing ores. However, due to environmental concerns, an intense search for a replacement of nonylphenol ethoxylates has been ongoing for a long time.

Thus, there is still a need for collector compositions having a better environmental profile than nonylphenol ethoxylates that perform equally well. Collector compositions aligned with this approach are described herein.

### DETAILED DESCRIPTION

. The Applicant has surprisingly found that employing a primary collector and a collector aid, and optionally a secondary collector, and conditioning a phosphate-containing ore with both these compounds in a froth flotation process will improve froth flotation results such as grade and recovery of the phosphate minerals during such froth flotation process. Further it has been found even more beneficial to pre-mix the primary collector and collector aid, and optionally a secondary collector (to form a collector composition) which will allow the collector composition to be added as a single product to the ore without the need for a separate conditioning step, while at the same time significantly improving the performance of the flotation.

Accordingly, the present invention relates to a process for froth flotation of an ore to recover phosphate-containing materials from the ore that includes adding a a primary collector and a collector aid to the ore and next performing a conditioning step of the ore in the presence of the primary collector and collector aid, wherein the primary collector is selected from the group consisting of an amphoteric surface-active compound, an anionic surface-active compound and combinations thereof; and the collector aid has the formula R³-CO-O-Aₙ-R⁴ where R³ is a linear or branched, alkyl or hydroxyalkyl group having from 3 to 8 carbon atoms, R⁴ is a linear or branched, alkyl or hydroxyalkyl group having from 3 to 10 carbon atoms, and at least one of R³ and R⁴ contains a hydroxyl group; and A is either ethoxy, propoxy or butoxy and n is a number from 0-10, wherein a ratio of the primary collector to the collector aid by weight is from 999:1 to 1:1.

The primary collector and the collector aid can be added to the ore one after the other or simultaneously in one collector composition. Preferably they are added to the ore pre-blended in one collector composition, which collector composition may optionally contain further compounds, such as for example a secondary collector compound.

The collector aid was found to boost the overall performance of the collector composition. The primary collector and collector aid in embodiments are contained in a single composition that is used for flotation or are added separately to be both present in the conditioning step. If an ore is conditioned with both the primary collector and the collector aid, the froth flotation results were found to be surprisingly better than when the collector aid component is added to the ore already conditioned with a composition that does not contain the collector aid of the present invention. In the direct flotation of apatite, for example, recovery can be improved by around 4% by weight using the collector composition to which the collector aid was initially pre-blended as neat compared to a process in which conditioning with the primary collector did not include the collector aid. Meanwhile, poor grade of P₂O₅ was observed when adding the collector aid after the conditioning of the ore as a frother. The collector composition containing both the primary collector and collector aid also yields better frothing characteristics, including improved froth density and stability.

It may be noted that in US2017/0252753 a process of froth flotating a phosphate-containing ore is disclosed employing a collector composition that contains an anionic or amphoteric primary collector in combination with a non-ionic ethoxylated alcohol as a secondary collector. In some of the embodiments, a frother is added to the process, that can be 2,2,4-trimethyl-1,3-pentanediol monoisobutyrate, but only after the ore was conditioned with the collector composition

The primary collector disclosed herein is an amphoteric surface-active compound, an anionic surface-active compound or a combination thereof. Surface-active compounds (or surfactants) are compounds that lower the surface tension or interfacial tension between two liquids, between a gas and a liquid, and/or between a solid and a liquid. Anionic surface-active compounds typically contain a negatively charged (anionic) head group. Amphoteric surface-active compounds contain both cationic (positively charged) and anionic moieties within the same molecule. Below some examples of the primary collectors are provided; these examples should only be considered as suitable and are not to be regarded as limiting.

In some embodiments the primary collector is an amphoteric surface-active compound having the formula (II) where R₁ is a hydrocarbyl group with 8-22, preferably 12-18, carbon atoms; A is an alkyleneoxy group having 2-4, preferably 2, carbon atoms; p is the number 0 or 1; q is a number from 0-5, preferably 0; R₂ is a hydrocarbyl group having 1-4, preferably 1, carbon atoms or R₂ is the group where R₁, A, p and q have the same meaning as above; Y⁻ is COOH or SO₃H, preferably COOH; n is the number 1 or 2, preferably 1; M is a cation, which can be monovalent or divalent and inorganic or organic, and r is the number 1 or 2. The primary collector can also be used in its acid form, where the nitrogen is protonated and no external cation is needed.

The compounds according to formula (II) can be produced from commercially available starting materials using known procedures. U.S. Patent No. 4,358,368 discloses some ways to produce the compounds where R₁ is a hydrocarbyl group with 8-22 carbon atoms (col. 6, line 9 - col. 7, line 52). U.S. Patent No. 4,828,687 (col. 2, line 2 - col. 2, line 31) describes compounds where R₂ is attached to the compound of formula (II) via the methylene group.

In other embodiments the primary collector has the formula (III) where R₂ is a hydrocarbyl group with 8-22, preferably 12-18, carbon atoms; D is -CH₂- or -CH₂CH₂-; k is a number from 0-4, preferably 0-3, and most preferably 0-2, and M is hydrogen or a cation such as sodium or potassium.

Compounds according to formula (III) are known and produced commercially by methods known in the art. Products where D is -CH₂- are prepared by the reaction between a fatty amine and chloroacetic acid or its salts, and products where D is -CH₂CH₂- are prepared by the reaction between a fatty amine and acrylic acid or esters thereof, in the latter case the reaction is followed by hydrolysis.

In still other embodiments the primary collector is an anionic surface-active compound, such as fatty acids having an alkyl group with 8-24 carbon atoms, sulfonates, alkyl phosphates, alkyl sulfates and compounds having the formula (IV) where R is a hydrocarbyl group having from 7-23, preferably 11-21, carbon atoms, optionally substituted; R₁ is H or CH₃, preferably H; R₂ is H or an alkyl group having from 1-4 carbon atoms, preferably H; R₃ is H or CH₃, preferably CH₃; n is a number from 0-20; p is a number from 1-3, preferably 1; X is H⁺ or a cation, organic or inorganic; and m represents the valency of the cation and is the number 1 or 2, preferably 1. The cation is preferably an alkali metal cation, an alkaline earth metal cation, ammonium, or a substituted ammonium group having one or more alkyl and/or hydroxyalkyl groups having from 1-3 carbon atoms.

For the production of compounds of formula (IV) see the description in WO2015/000931 (corresponding to PCT/EP2014/064014).

Preferably, the primary collector comprises a sodium salt of an alkyl glycinate or sarcosinate having from 12 to 20, more preferably 12 to 16 carbon atoms. In one particular embodiment, the primary collector is N-[2-hydroxy-3-(C12-16-alkyloxy)propyl]-N-methyl glycinate (sodium C14-C15 sarcosinate).

Suitable fatty acids having an alkyl group with 8-24 carbon atoms include fatty acids based on tall oil and oils of safflower, sunflower, soya, raps, corn, lineseed, rapeseed, tallow, coconut, raw coniferous, and raw foliar).

In other embodiments the primary collector is a phosphate ester. In one embodiment, phosphate esters have the formulas
R²-(O-CH₂-CH₂)ₙ-O-P(O)(OM)-O-P(O)(OM)-(O-CH₂-CH₂)ₙ-O-R², R²-(O-CH₂-CH₂)ₙ-O-PO(OM)₂ or (R²-(O-CH₂-CH₂)ₙ-O)₂-PO-OM or a combination of thereof where R² is an alkyl group having from 6-22 carbon atoms, preferably 16-18 carbon atoms; n is a number from 0-25 preferably 4; and M is a monovalent cation such as sodium or hydrogen. Alcohol ethoxylate phosphate ester (Phospholan type, Akzo Nobel Surface Chemistry LLC) contains the above phosphate esters where R² is an alkyl group having 18 carbon atoms, n is 4, and M is sodium or hydrogen.

Other suitable phosphate esters are monophosphate and diphosphate esters containing from 6-22 carbon atoms (linear or branched, degree of branching 1-3) and from 0-25 ethylene oxide (EO) units, and combination thereof. "Degree of branching" as used herein means the total number of methyl groups present on the main alkyl chain minus one.

The collector aid of the collector composition is an ester having the formula

R³-CO-O-Aₙ-R⁴

where R³ is a linear or branched, alkyl or hydroxyalkyl group having from 3 to 8 carbon atoms, R⁴ is a linear or branched, alkyl or hydroxyalkyl group having from 3 to 10 carbon atoms, and at least one of R³ and R⁴ contains a hydroxyl group; and A is either ethoxy, propoxy or butoxy and n is a number from 0-10. Below some examples of the collector aids are provided; these examples should only be considered as suitable and are not to be regarded as limiting.

Suitable collector aids include 2,2,4-trimethyl-1,3-pentanediol monoisobutyrate (Eastman Chemical Company); pentanoic acid, 3-hydroxy-4,4-dimethyl-2-(1-methylethyl)-, ethyl ester; heptanoic acid, 3-hydroxy-2,2,4-trimethyl-, ethyl ester; hexanoic acid, 4-ethyl-3-hydroxy-2,2-dimethyl-, ethyl ester; 2-ethylhexane-(1,3)-diol mono-n-butyrate; 2-ethylhexane-(1,3)-diol di-n-butyrate, alkoxylated derivatives of same containing from 0-10 alkoxy units (more preferably 0-3 ethoxy units or 0-10 propoxy units), and combinations thereof.

The weight ratio between the primary collector and the collector aid is from 999:1 to 1:1, preferably from 99:1 to 95:5, and more preferably from 99:1 to 96:4. All weight ratios herein refer to the ratio of active materials, unless stated otherwise.

The collector composition containing the primary collector and the collector aid can optionally include a solvent. The role of the solvent in the collector composition is to improve the flotation froth quality and the liquidity of the final formulation. Suitable solvents include ethoxylated alcohols having from 3 to 10 EO groups, glycols (e.g., propylene glycol, diethylene glycol, etc.), non-ionic surfactants, low molecular weight alcohols, such C1-C15 alcohols, low molecular weight organic acids, such as C1-C15 organic acids, low molecular weight ethanolamines (e.g., triethanolamine, methyl diethanolamine, diethanolamine, etc.), water, organic solvents (*e.g.*, toluene, hexane, etc.), aliphatic hydrocarbons, such as isoparaffines, paraffines, cycloparaffines, and their combinations. Low molecular weight solvents are in a preferred embodiment defined as solvents that have a molecular weight of up to 120 g/mole. The weight ratio between the primary collector and the optional solvent is preferably from 999:1 to 80:20, preferably from 99:1 to 90:10.

The collector composition may be prepared by adding the primary collector, the collector aid and the optional solvent to a suitable vessel and mixing to combine. Additional flotation aids described herein can also be added to the collector composition before or after the primary collector and collector aid are combined. No special preparation steps (e.g., high shear mixing, heating, etc.) are necessary to prepare the collector composition.

This disclosure also describes a process for the froth flotation of non-sulfidic ores, especially phosphate ores, to recover apatite minerals, in which process the collector composition described herein is used. Such froth flotation process for phosphate ores can typically include the following steps: a) conditioning a pulped phosphate-containing ore, wherein the ore includes a phosphate-containing mineral, and gangue minerals, with an effective amount of the collector composition described herein or the primary collector and collector aid separately, and optionally other flotation aids, and b) performing a froth flotation process to recover the phosphate-containing mineral(s).

The amount of primary collector added to the ore will in general be in the range of from 10 to 1000 g/ton dry ore, preferably in the range of from 20 to 500 g/ton dry ore, more preferably from 100 to 400 g/ton dry ore. The amount of collector aid to added to the ore will in general be in the range of from 0.01-50 g/ton dry ore, preferably in the range of from 0.02-25 g/ton dry ore, more preferably from 0.05-20 g/ton dry ore

In preferred embodiments a secondary collector can be present during the conditioning step. In more preferred embodiments the secondary collector is selected from the group of anionic collector compounds, non-ionic collector compounds or mixtures of two or more of those, wherein the anionic collector is selected from the group of fatty acids, alkylsulfosuccinates, alkylmaleates, alkylamidecarboxylate, esters of alkylamidecarboxylates, alkylbenzenesulphonates, alkylsulfonates, and sulfonated fatty acids, and the non-ionic collector compound is selected from the group of ethoxylates, glycosides, and ethanolamides, most preferably the non-ionic collector compound is selected from the group of branched and unbranched ethoxylated C11-C24 alcohols, ethoxylated C10-C24 alkylamines, sugar surfactants, ethoxylated C10-C24 fatty acids

Further flotation aids that can be present in the flotation process are depressants such as a polysaccharide, alkalized starch or dextrin; extender oils; frothers/froth regulators such as pine oil, MIBC (methylisobutyl carbinol) and alcohols such as hexanol and alcohol ethoxylates/propoxylates, preferably C6-C10 alcohols and ethoxylates thereof; inorganic dispersants such as silicate of sodium (water glass) and soda ash; and pH-regulators (which can be acidic or alkaline compounds to adjust the pH as desired). These flotation aids can be added to the collector composition or added to the flotation process before or following conditioning of the ore with the primary collector and collector aid, optionally preblended in a collector composition.

The present invention in a preferred embodiment relates to a process for froth flotation of a phosphate ore, the process comprising: optionally, adding a depressant to the ore; adding the primary collector and collector aid as above to the ore; optionally, adding one or more further components to the ore selected from the group of pH adjusting agents, dispersants and secondary collector; wherein the primary collector, the collector aid and optional secondary collector can be added one after the other or simultaneously, optionally preblended in one collector composition; conditioning the ore in the presence of the primary collector, optional secondary collector, and the collector aid; subsequently, optionally adding one or more further components to the conditioned ore selected from the group of pH adjusting agents, dispersants and frothers; and performing a froth flotation process to recover phosphate-containing materials from the ore.

In a preferred embodiment of the process of the invention, in a step subsequent to the conditioning of the ore in the presence of the primary collector and collector aid, a frother is added to the conditioned ore.

The pH during the flotation process will normally be in the range of pH 8-11.

### EXAMPLES

For all Examples, a phosphate ore containing 42% apatite, 38% nepheline, 5% aegirine, 3% feldspar and 2% sphene was crushed and ground to a desirable flotation size (70% -160 µm). In each Example, 500 g of the phosphate ore was placed into a 1.3 L (for rougher), 1.0 L (for cleaner 1) or 0.5 L (for cleaner 2) flotation cell. Tap water (Stenungsund municipal water with hardness 4 °dH) was added to the marked level in the cell (1.4L) and mixing was started. Further, 200 g/t water glass as a 1 wt-% solution was added and conditioned for 1 minute. In each Example flotation was performed at room temperature (20±1 °C), and the rougher flotation, the cleaner 1 flotation and the cleaner 2 flotation were performed for 4 minutes, 3 minutes and 2 minutes, respectively. All fractions (tailings, middlings and concentrate) were collected and analysed. For each Example, alcohol ethoxylate phosphate ester (Phospholan type, Akzo Nobel Surface Chemistry LLC, henceforth "Phosphate Ester") is a phosphate ester having the general formula R²-(O-CH₂-CH₂)ₙ-O-PO(OM)₂ and (R²-(O-CH₂-CH₂)ₙ-O)₂-PO-OM where R² is an alkyl group having 18 carbon atoms, n is 4, and M is sodium or hydrogen.

### Example 1(Comparative): Collectors added individually- No collector aid

Separate 1 wt-% solutions were prepared for each of tall oils, alkylbenzene sulfonate and Phosphate Ester.

The pH of the flotation mixture was adjusted to 9.9 with a 5% aqueous NaOH solution and quantities of the 1 wt-% solutions of the tall oils, alkylbenzene sulfonate and Phosphate Ester were added to the flotation cell to be equivalent to 150 g/t of a collector composition containing 50 wt-% tall oils, 17 wt-% alkylbenzene sulfonate, and 33 wt-% Phosphate Ester. A conditioning step was carried out at 1000 rpm and room temperature for two minutes. After the conditioning step, the flotation (1000 rpm and 3 L/min rougher; 1500 rpm and 1.3 L/min cleaner 1; and 1500 rpm and 0.6 L/min cleaner 2) was started. The flotation results are shown in Table 1.

**Table 1**

| Collector | Flotation Stage | P₂O₅ Recovery (%) | P₂O₅ Grade (%) |
|---|---|---|---|
| 150 g/t: 50 wt-% tall oils, 17 wt-% alkylbenzene sulfonate, 33 wt-% Phosphate Ester (1 wt-% solutions, added separately) | Rougher | 97.2 | 29.7 |
| | Cleaner 1 | 90.3 | 37.5 |
| | Cleaner 2 | 82.3 | 39.8 |

### Example 2 (Comparative): Collectors pre-mixed - No collector aid

A collector composition containing 50 wt-% tall oils, 17 wt-% alkylbenzene sulfonate, and 33 wt-% Phosphate Ester was prepared. The collector composition was diluted in deionized water to a 1 wt-% solution.

The pH of the flotation mixture was adjusted to 9.9 with a 5% aqueous NaOH solution and 150 g/t of the collector composition as a 1 wt-% aqueous solution was added to the flotation cell. A conditioning step was carried out at 1000 rpm and room temperature for two minutes. After the conditioning step, the flotation (1000 rpm and 3 L/min rougher; 1500 rpm and 1.3 L/min cleaner 1; and 1500 rpm and 0.6 L/min cleaner 2) was started. The flotation results are shown in Table 2.

**Table 2**

| Collector | Flotation Stage | P₂O₅ Recovery (%) | P₂O₅ Grade (%) |
|---|---|---|---|
| 150 g/t: 50 wt-% tall oils, 17 wt-% alkylbenzene sulfonate, 33 wt-% Phosphate Ester (1 wt-% solution, pre-mixed) | Rougher | 95.8 | 30.9 |
| | Cleaner 1 | 88.9 | 38.2 |
| | Cleaner 2 | 81.1 | 39.8 |

The Example 1 and Example 2 results show, in the absence of the collector aid, a collector composition in which the composition components were separately added to the flotation showed no significant differences with respect to the same collector composition in which the components were pre-mixed and added to the flotation all at once.

### Example 3 (Comparative): Collector aid added as frother after conditioning

The pH of the flotation mixture was adjusted to 9.9 with a 5% aqueous NaOH solution and quantities of the 1 wt-% solutions of tall oils and Phosphate Ester (the same as in Example 1) were mixed together and added to the flotation cell as a single stock solution to be equivalent to 145.5 g/t of a collector composition containing 61.8 wt-% tall oils and 38.2 wt-% Phosphate Ester. A conditioning step was carried out at 1000 rpm and room temperature for two minutes. After the conditioning step, 4.5 g/t of collector aid (2,2,4-trimethyl-1,3-pentanediol monoisobutyrate) was added and the flotation (1000 rpm and 3 L/min rougher; 1500 rpm, 1.3 L/min cleaner 1; and 1500 rpm and 0.6 L/min cleaner 2) was started. The flotation results are shown in Table 3.

**Table 3**

| Collector | Flotation Stage | P₂O₅ Recovery (%) | P₂O₅ Grade (%) |
|---|---|---|---|
| 150 g/t: 60 wt-% tall oils, 37 wt-% phosphate ester (added to conditioning as single stock solution) and 3 wt-% collector aid (added after the conditioning as a frother) | Rougher | 98.7 | 22.7 |
| | Cleaner 1 | 97 | 31.8 |
| | Cleaner 2 | 95.8 | 35.6 |

When the collector aid was added as a frother after conditioning the ore with the collectors, the grade of P₂O₅ dropped below the acceptable level of 39.0%.

### Example 4: Collector aid, pre-mixed with primary collector

A collector composition containing 60 wt-% tall oils, 37 wt-% Phosphate Ester, and 3 wt-% collector aid (2,2,4-trimethyl-1,3-pentanediol monoisobutyrate) was prepared. The collector composition was diluted in deionized water to a 1 wt-% solution.

The pH of the flotation mixture was adjusted to 9.9 with a 5% aqueous NaOH solution and 150 g/t of the collector composition as a 1 wt-% aqueous solution was added to the flotation cell. A conditioning step was carried out at 1000 rpm and room temperature for two minutes. After the conditioning step, the flotation (1000 rpm and 3 L/min rougher; 1500 rpm and 1.3 L/min cleaner 1; and 1500 rpm and 0.6 L/min cleaner 2) was started. The flotation results are shown in Table 4.

**Table 4**

| Collector | Flotation Stage | P₂O₅ Recovery (%) | P₂O₅ Grade (%) |
|---|---|---|---|
| 150 g/t: 60 wt-% tall oils, 37 wt-% phosphate ester, and 3 wt-% collector aid (1 wt-% solution, pre-mixed) | Rougher | 96.3 | 30.1 |
| | Cleaner 1 | 92.3 | 38.5 |
| | Cleaner 2 | 86.5 | 40.4 |

Grade and recovery were improved over a collector composition having comparable levels of the other collectors but without the collector aid (Example 2).

As one can see from the results above, collector compositions containing the collector aid described herein (*e.g.*, 2,2,4-trimethyl-1,3-pentanediol monoisobutyrate) showed improved grade and/or recovery from flotation when compared to collector compositions that did not contain the collector aid and to compositions in which the collector aid was added (as a frother) at a later step in the flotation, namely after the conditioning of the ore. The results clearly show that the presence of the collector aid in the collector composition at the start of the flotation process plays a crucial role in the flotation.

### Example 5: Collector aid added to conditioning separately

The pH of the flotation mixture was adjusted to 9.9 with a 5% aqueous NaOH solution and quantities of the 1 wt-% solutions of tall oils and Phosphate Ester (the same as in Example 1) were mixed together and added to the flotation cell to be equivalent to 145.5 g/t of a collector composition containing 61.8 wt-% tall oils and 38.2 wt-% Phosphate Ester. The collector aid (2,2,4-trimethyl-1,3-pentanediol monoisobutyrate) was added to the conditioning step separately from the main collector stock solution to be equivalent to 4.5 g/t. A conditioning step was carried out at 1000 rpm and room temperature for two minutes. The flotation (1000 rpm and 3 L/min rougher; 1500 rpm, 1.3 L/min cleaner 1; and 1500 rpm and 0.6 L/min cleaner 2) was started. The flotation results are shown in Table 5.

**Table 5**

| Collector | Flotation Stage | P₂O₅ Recovery (%) | P₂O₅ Grade (%) |
|---|---|---|---|
| 150 g/t: 60 wt-% tall oils, 37 wt-% phosphate ester (added to conditioning as collector stock solution #1) and 3 wt-% collector aid (added to conditioning separately as additive #2) | Rougher | 98.8 | 26.9 |
| | Cleaner 1 | 96.8 | 34.7 |
| | Cleaner 2 | 95.5 | 37.4 |

This Example 5 shows that when the collector was added separately from the main collector solution before the conditioning step of the ore, the grade of P₂O₅ remained higher than in the Example 3 demonstrating that the collector aid if present during the conditioning step improves the results. Pre-blending the collector aid with the other collector compounds is however preferred as visible from the results obtained in Example 4.

## Claims

1. Process for froth flotation of an ore to recover phosphate-containing materials from the ore that includes adding a primary collector and a collector aid to the ore, next performing a conditioning step of the ore, wherein:
the primary collector is selected from the group consisting of an amphoteric surface-active compound, an anionic surface-active compound and combinations thereof; and
the collector aid has the formula
R³-CO-O-Aₙ-R⁴
where R³ is a linear or branched, alkyl or hydroxyalkyl group having from 3 to 8 carbon atoms, R⁴ is a linear or branched, alkyl or hydroxyalkyl group having from 3 to 10 carbon atoms, and at least one of R³ and R⁴ contains a hydroxyl group; A is either ethoxy, propoxy or butoxy and n is 0-10,
wherein a ratio of the primary collector to the collector aid by weight is from 999:1 to 1:1.

2. The process of claim 1 wherein the primary collector and collector aid are blended before they are added to the ore.

3. The process of claim 1 or 2, wherein the primary collector is selected from the group consisting of:
a compound having the formula
where R₁ is a hydrocarbyl group with 8-22, preferably 12-18, carbon atoms; A is an alkyleneoxy group having 2-4, preferably 2, carbon atoms; p is the number 0 or 1; q is a number from 0-5, preferably 0; R₂ is a hydrocarbyl group having 1-4, preferably 1, carbon atoms or R₂ is the group
where R₁, A, p and q have the same meaning as above; Y⁻ is COOH or SO₃H, preferably COOH; n is the number 1 or 2, preferably 1; M is a cation, which can be monovalent or divalent, and inorganic or organic, and r is the number 1 or 2; a compound having the formula
where R₂ is a hydrocarbyl group with 8-22, preferably 12-18, carbon atoms; D is -CH₂- or -CH₂CH₂- ; k is a number from 0-4, preferably 0-3, and most preferably 0-2, and M is hydrogen or a cation;
a compound having the formula
where R is a hydrocarbyl group having from 7-23, preferably 11-21, carbon atoms, optionally substituted; R₁ is H or CH₃, preferably H; R₂ is H or an alkyl group having from 1-4 carbon atoms, preferably H; R₃ is H or CH₃, preferably
CH₃; n is a number from 0-20; p is a number from 1-3, preferably 1; X is H⁺ or a cation, organic or inorganic; and m represents the valency of the cation and is the number 1 or 2, preferably 1;
a phosphate ester having the formula
R²-(O-CH₂-CH₂)ₙ-O-P(O)(OM)-O-P(O)(OM)-(O-CH₂-CH₂)ₙ-O-R², R²-(O-CH₂-CH₂)ₙ-O-PO(OM)₂ or (R²-(O-CH₂-CH₂)ₙ-O)₂-PO-OM or combination of thereof where R² is an alkyl group having from 6 to 22, preferably 16-18, carbon atoms, n is a number from 0 to 10, and M is a monovalent cation or hydrogen;
a fatty acid having from 8 to 24 carbon atoms; and combinations thereof.

4. The process of any one of claims 1 to 3, wherein the primary collector comprises a sodium salt of an alkyl glycinate or alkyl sarcosinate, the alkyl having from 12 to 20, preferably 12 to 16 carbon atoms.

5. The process of any one of claims 1 to 3, wherein the primary collector is N-[2-hydroxy-3-(C12-16-alkyloxy)propyl]-N-methyl glycinate.

6. The process of any one of claims 1 to 3, wherein the primary collector is a phosphate ester having the formula
R²-(O-CH₂-CH₂)ₙ-O-PO(OM)₂ or (R²-(O-CH₂-CH₂)ₙ-O)₂-PO-OM or a combination thereof
where R² is an alkyl group having 18 carbon atoms, n is 4, and M is sodium or hydrogen.

7. The process of any one of claims 1 to 3, wherein the primary collector is tall oil fatty acid.

8. The process of any one of claims 1 to 7, wherein the collector aid is 2,2,4-trimethyl-1,3-pentanediol monoisobutyrate.

9. The process of any preceding claim, wherein a ratio of the primary collector to the collector aid by weight is from 99:1 to 95:5, and preferably from 99:1 to 96:4.

10. The process of any preceding claim, further comprising a solvent, wherein the solvent is preferably selected from the group consisting of ethoxylated alcohols having from 3 to 10 EO groups, glycols, non-ionic surfactants, C1-C15 alcohols, C1-C15 organic acids, ethanolamines, water, organic solvents, aliphatic hydrocarbons and combinations thereof.

11. The process of claim 10, wherein a ratio of the primary collector to the solvent by weight is from 999:1 to 80:20.

12. The process of any one of claims 1 to 11 wherein a frother is added during the froth flotation step in a step subsequent to conditioning the ore.

13. The process for froth flotation of a phosphate ore of any one of claims 1 to 12, the process comprising:
optionally, adding a depressant to the ore;
adding the primary collector and collector aid, of any of claims 1 through 12 to the ore;
optionally, adding one or more further components to the ore selected from the group of pH adjusting agents, dispersants and secondary collector;
wherein the primary collector, the collector aid and optional secondary collector can be added one after the other or simultaneously;
conditioning the ore in the presence of the primary collector, optional secondary collector, and the collector aid;
subsequently, optionally adding one or more further components to the conditioned ore selected from the group of pH adjusting agents, dispersants and frothers;
and
performing a froth flotation process to recover phosphate-containing materials from the ore.

14. The process of claim 13, wherein the secondary collector is selected from the group of anionic collector compounds, non-ionic collector compounds or mixtures of two or more of those, wherein the anionic collector compound is selected from the group of fatty acids, alkylsulfosuccinates, alkylmaleates, alkylamidocarboxylates, esters of alkylamidocarboxylates, alkylbenzensulphonates, alkylsulfonates, and sulphonated fatty acids and the nonionic collector compound is selected from the group of ethoxylates, glycosides, and ethanolamides, preferably the non-ionic collector compound is selected from the group of branched and unbranched ethoxylated C11-C24 alcohols, ethoxylated C10-C24 alkylamines, sugar surfactants, ethoxylated C10- C24 fatty acids.

15. Process of claim 13 or 14 wherein the frother is selected from the group of pineoils, MIBC (methylisobutyl carbinal) and alcohols and alcohol ethoylates, preferably C6-C10 alcohols and ethoxylates thereof.

## Patentansprüche

1. Verfahren für die Schaumflotation eines Erzes, um phosphathaltige Materialien aus dem Erz zu gewinnen, das das Zusetzen eines primären Sammlers und einer Sammlerhilfe zu dem Erz, als nächstes das Ausführen eines Konditionierschritts des Erzes umfasst, wobei:
der primäre Sammler aus der Gruppe ausgewählt wird bestehend aus einer amphoteren oberflächenaktiven Verbindung, einer anionischen oberflächenaktiven Verbindung und einer Kombination davon; und
die Sammlerhilfe die Formel
R³-CO-O-Aₙ-R⁴
aufweist, wobei R³ eine lineare oder verzweigte Alkyl- oder Hydroxyalkylgruppe ist, die 3 bis 8 Kohlenstoffatome aufweist, R⁴ eine lineare oder verzweigte Alkyl- oder Hydroxyalkylgruppe ist, die 3 bis 8 Kohlenstoffatome aufweist, und mindestens eines von R³ und R⁴ eine Hydroxylgruppe enthält; A entweder Ethoxy, Propoxy oder Butoxy ist und n 0-10 beträgt,
wobei ein Verhältnis des primären Sammlers zu der Sammlerhilfe, auf das Gewicht bezogen, 999:1 bis 1:1 beträgt.

2. Verfahren nach Anspruch 1, wobei der primäre Sammler und die Sammlerhilfe vermischt werden, bevor sie dem Erz zugesetzt werden.

3. Verfahren nach Anspruch 1 oder 2, wobei der primäre Sammler aus der Gruppe ausgewählt wird bestehend aus:
einer Verbindung, die die Formel
aufweist, wobei R₁ eine Hydrocarbylgruppe mit 8-22, bevorzugt 12-18 Kohlestoffatomen ist; A eine Alkylenoxygruppe ist, die 2-4, bevorzugt 2 Kohlenstoffatome aufweist; p die Zahl 0 oder 1 ist; q eine Zahl von 0-5, bevorzugt 0 ist; R₂ eine Hydrocarbylgruppe ist, die 1-4, bevorzugt 1 Kohlenstoffatom aufweist oder R₂ die Gruppe ist, wobei R₁, A, p und q dieselbe Bedeutung wie oben aufweisen; Y⁻ COOH oder SO₃H, bevorzugt COOH ist; n die Zahl 1 oder 2, bevorzugt 1 ist; M ein Kation ist, das einwertig oder zweiwertig und anorganisch oder organisch sein kann, und r die Zahl 1 oder 2 ist;
einer Verbindung, die die Formel aufweist
wobei R₂ eine Hydrocarbylgruppe mit 8-22, bevorzugt 12-18 Kohlenstoffatomen ist; D -CH₂- oder -CH₂CH₂- ist; k eine Zahl von 0-4, bevorzugt 0-3 und am bevorzugtesten 0-2 ist und M Wasserstoff oder ein Kation ist;
einer Verbindung, die die Formel aufweist
wobei Reine Hydrocarbylgruppe ist, die 7-23, bevorzugt 11-21 Kohlenstoffatome, die wahlweise substituiert sind, aufweist; R₁ H oder CH₃, bevorzugt H ist; R₂ H oder eine Alkylgruppe, die 1-4 Kohlenstoffatome aufweist, bevorzugt H ist; R₃ H oder CH₃, bevorzugt CH₃ ist; n eine Zahl von 0-20 ist; p eine Zahl von 1-3, bevorzugt 1 ist; X H⁺ oder ein Kation, organisch oder anorganisch ist; und m die Wertigkeit des Kations darstellt und die Zahl 1 oder 2, bevorzugt 1 ist;
einem Phosphatester, der die Formel aufweist
R²-(O-CH₂-CH₂)ₙ-O-P(O)(OM)-O-P(O)(OM)-(O-CH₂-CH₂)ₙ-O-R², R²-(O-CH₂-CH₂)ₙ-O-PO(OM)₂ oder R²-(O-CH₂-CH₂)ₙ-O)₂-PO-OM oder eine Kombination davon,
wobei R² eine Alkylgruppe ist, die 6 bis 22, bevorzugt 16-18 Kohlenstoffatome aufweist, n eine Zahl von 0 bis 10 ist und M ein einwertiges Kation oder Wasserstoff ist;
einer Fettsäure, die 8 bis 24 Kohlenstoffatome aufweist; und Kombinationen davon.

4. Verfahren nach einem der Ansprüche 1 bis 3, wobei der primäre Sammler ein Natriumsalz eines Alkylglycinats oder Alkylsarcosinats umfasst, wobei das Alkyl 12 bis 20, bevorzugt 12 bis 16 Kohlenstoffatome aufweist.

5. Verfahren nach einem der Ansprüche 1 bis 3, wobei der primäre Sammler N-[2-Hydroxy-3-(C12-16-alkyloxy)propyl]-N-methylglycinat ist.

6. Verfahren nach einem der Ansprüche 1 bis 3, wobei der primäre Sammler ein Phosphatester ist, der die Formel
R²-(O-CH₂-CH₂)ₙ-O-PO(OM)₂ oder R²-(O-CH₂-CH₂)ₙ-PO-OM oder eine Kombination davon aufweist,
wobei R²eine Alkylgruppe ist, die 18 Kohlenstoffatome aufweist, n 4 beträgt und M Natrium oder Wasserstoff ist.

7. Verfahren nach einem der Ansprüche 1 bis 3, wobei der primäre Sammler Tallöl oder Fettsäure ist.

8. Verfahren nach einem der Ansprüche 1 bis 7, wobei die Sammlerhilfe 2,2,4-Trimethyl-1,3-pentandiolmonoisobutyrat ist.

9. Verfahren nach einem vorhergehenden Anspruch, wobei ein Verhältnis des primären Sammlers zu der Sammlerhilfe, auf das Gewicht bezogen, 99:1 bis 95:5 und bevorzugt 99:1 bis 96:4 beträgt.

10. Verfahren nach einem vorhergehenden Anspruch, ferner ein Lösungsmittel umfassend wobei das Lösungsmittel bevorzugt aus der Gruppe ausgewählt ist bestehend aus ethoxylierten Alkoholen, die 3 bis 10 EO-Gruppen aufweisen, Glycolen, nichtionischen Tensiden, C1-C15-Alkoholen, organischen C1-C15-Säuren, Ethanolaminen, Wasser, organischen Lösungsmitteln, aliphatischen Kohlenstoffatomen und Kombinationen davon.

11. Verfahren nach Anspruch 10, wobei ein Verhältnis des primären Sammlers zu dem Lösungsmittel, auf das Gewicht bezogen, 999:1 bis 80:20 beträgt.

12. Verfahren nach einem der Ansprüche 1 bis 11, wobei ein Schäumer während des Schaumflotationsschritts in einem auf das Konditionieren des Erzes folgenden Schritt zugegeben wird.

13. Verfahren für die Schaumflotation eines Phosphaterzes nach einem der Ansprüche 1 bis 12, wobei das Verfahren Folgendes umfasst:
wahlweise Zusetzen eines Dämpfungsmittels zu dem Erz;
Zusetzen des primären Sammlers und der Sammlerhilfe nach einem der Ansprüche 1 bis 12 zu dem Erz;
wahlweise Zusetzen einer oder mehrerer weiterer Komponenten zu dem Erz ausgewählt aus der Gruppe von pH-Wert-Einstellungsmitteln, Dispergiermitteln und sekundärem Sammler;
wobei der primäre Sammler, die Sammlerhilfe und der wahlweise sekundäre Sammler einer nach dem anderen oder gleichzeitig zugegeben werden können;
Konditionieren des Erzes in Gegenwart des primären Sammlers, des wahlweisen sekundären Sammlers und der Erstsammlerhilfe;
daraufhin wahlweise Zusetzen, zu dem konditionierten Erz, einer oder mehrerer weiterer Komponenten ausgewählt aus der Gruppe von pH-Wert-Einstellungsmitteln, Dispergiermitteln und Schäumern;
und
Ausführen eines Schaumflotationsvorgangs, um phosphathaltige Materialien aus dem Erz zu gewinnen.

14. Verfahren nach Anspruch 13, wobei der sekundäre Sammler aus der Gruppe ausgewählt wird von anionischen Sammlerverbindungen, nichtionischen Sammlerverbindungen oder Mischungen von zwei oder mehr dieser, wobei die anionische Sammlerverbindung aus der Gruppe ausgewählt wird von Fettsäuren, Alkylsulfosuccinaten, Alkylmaleaten, Alkylamidcarboxylaten, Estern von Alkylamidcarboxylaten, Alkylbenzolsulfonaten, Alkylsulfonaten und sulfonierten Fettsäuren und die nichtionische Sammlerverbindung aus der Gruppe ausgewählt wird von Ethoxylaten, Glycosiden und Ethanolamiden, die nichtionische Sammlerverbindung bevorzugt aus der Gruppe ausgewählt wird von verzweigten und unverzweigten ethoxylierten C11-C24-Alkoholen, ethoxylierten C10-C24-Alkylaminen, Zuckertensiden, ethoxylierten C10-C24-Fettsäuren.

15. Verfahren nach Anspruch 13 oder 14, wobei der Schäumer aus der Gruppe ausgewählt wird von Kiefernölen, MIBC (Methylisobutylcarbinal) und Alkoholen und Alkoholethoxylaten, bevorzugt C6-C10-Alkoholen und Ethoxylaten davon.

## Revendications

1. Procédé de flottation par mousse d'un minerai pour récupérer les matériaux contenant du phosphate du minerai, qui comprend l'ajout d'un collecteur primaire et d'un auxiliaire pour le collecteur au minerai, puis la mise en oeuvre d'une étape de conditionnement du minerai, dans lequel :
le collecteur primaire est sélectionné dans le groupe constitué par un composé tensioactif amphotère, un composé tensioactif anionique et des combinaisons de ceux-ci ; et
l'auxiliaire pour le collecteur répond à la formule
R³-CO-O-Aₙ-R⁴
où R³ est un groupe alkyle ou hydroxyalkyle, linéaire ou ramifié ayant de 3 à 8 atomes de carbone, R⁴ est un groupe alkyle ou hydroxyalkyle, linéaire ou ramifié ayant de 3 à 10 atomes de carbone et au moins l'un parmi R³ et R⁴ contient un groupe hydroxyle ; A est un groupe éthoxy, propoxy ou butoxy et n vaut 0 à 10,
dans lequel un rapport en poids du collecteur primaire à l'auxiliaire pour le collecteur est de 999:1 à 1:1.

2. Procédé selon la revendication 1, dans lequel le collecteur primaire et l'auxiliaire pour le collecteur sont mélangés avant d'être ajoutés au minerai.

3. Procédé selon la revendication 1 ou 2, dans lequel le collecteur primaire est sélectionné dans le groupe constitué par :
un composé répondant à la formule
où R₁ est un groupe hydrocarbyle ayant 8 à 22, de préférence 12 à 18 atomes de carbone ; A est un groupe alkylèneoxy ayant 2 à 4, de préférence 2, atomes de carbone ; p est le nombre 0 ou 1 ; q est un nombre de 0 à 5, de préférence 0 ; R₂ est un groupe hydrocarbyle ayant 1 à 4, de préférence 1, atomes de carbone ou R₂ est le groupe
où R₁, A, p et q ont la même signification que ci-dessus ; Y⁻ est COOH ou SO₃H, de préférence COOH ; n est le nombre 1 ou 2, de préférence 1 ; M est un cation, qui peut être monovalent ou divalent, et inorganique ou organique, et r est le nombre 1 ou 2 ;
un composé répondant à la formule
où R₂ est un groupe hydrocarbyle ayant 8 à 22, de préférence 12 à 18 atomes de carbone ; D est -CH₂- ou -CH₂CH₂- ; k est un nombre de 0 à 4, de préférence de 0 à 3, et de manière préférée entre toutes de 0 à 2, et M est un atome d'hydrogène ou un cation ;
un composé répondant à la formule
où R est un groupe hydrocarbyle ayant de 7 à 23, de préférence de 11 à 21 atomes de carbone, éventuellement substitué ; R₁ est H ou CH₃, de préférence H ; R₂ est H ou un groupe alkyle ayant de 1 à 4 atomes de carbone, de préférence H ; R₃ est H ou CH₃, de préférence CH₃ ; n est un nombre de 0 à 20 ; p est un nombre de 1 à 3, de préférence 1 ; X est H⁺ ou un cation, organique ou inorganique ; et m représente la valence du cation et est le nombre 1 ou 2, de préférence 1 ;
un ester de phosphate répondant à la formule
R²-(O-CH₂-CH₂)ₙ-O-P(O)(OM)-O-P(O)(OM)-(O-CH₂-CH₂)ₙ-O-R², R²-(O-CH₂-CH₂)ₙ-O-PO(OM)₂ ou (R²-(O-CH₂-CH₂)ₙ-O)₂-PO-OM ou une combinaison de ceux-ci, où R² est un groupe alkyle ayant de 6 à 22, de préférence 16 à 18 atomes de carbone, n est un nombre de 0 à 10 et M est un cation monovalent ou un hydrogène ;
un acide gras ayant de 8 à 24 atomes de carbone ; et des combinaisons de ceux-ci.

4. Procédé selon l'une quelconque des revendications 1 à 3, dans lequel le collecteur primaire comprend un sel de sodium d'un glycinate d'alkyle ou d'un sarcosinate d'alkyle, l'alkyle ayant de 12 à 20, de préférence 12 à 16 atomes de carbone.

5. Procédé selon l'une quelconque des revendications 1 à 3, dans lequel le collecteur primaire est le glycinate de N-[2-hydroxy-3-(alkyloxy en C12-16)propyl]-N-méthyle.

6. Procédé selon l'une quelconque des revendications 1 à 3, dans lequel le collecteur primaire est un ester de phosphate répondant à la formule
R²-(O-CH₂-CH₂),,-O-PO(OM)₂ ou (R²-(O-CH₂-CH₂)ₙ-O)₂-PO-OM ou une combinaison de ceux-ci
où R² est un groupe alkyle ayant 18 atomes de carbone, n vaut 4 et M est un atome de sodium ou un atome d'hydrogène.

7. Procédé selon l'une quelconque des revendications 1 à 3, dans lequel le collecteur primaire est un acide gras de tallöl.

8. Procédé selon l'une quelconque des revendications 1 à 7, dans lequel l'auxiliaire pour le collecteur est le monoisobutyrate de 2,2,4-triméthyl-1 ,3-pentanediol.

9. Procédé selon l'une quelconque des revendications précédentes, dans lequel un rapport en poids du collecteur primaire à l'auxiliaire pour le collecteur est de 99:1 à 95:5, de préférence de 99:1 à 96:4.

10. Procédé selon l'une quelconque des revendications précédentes, comprenant en outre un solvant, dans lequel le solvant est de préférence sélectionné dans le groupe constitué par les alcools éthoxylés ayant de 3 à 10 groupes EO, les glycols, les tensioactifs non ioniques, les alcools en C1 à C15, les acides organiques en C1 à C15, les éthanolamines, l'eau, les solvants organiques, les hydrocarbures aliphatiques et des combinaisons de ceux-ci.

11. Procédé selon la revendication 10, dans lequel le rapport en poids du collecteur primaire au solvant est de 999:1 à 80:20.

12. Procédé selon l'une quelconque des revendications 1 à 11, dans lequel un agent moussant est ajouté pendant l'étape de flottation par mousse dans une étape ultérieure au conditionnement du minerai.

13. Procédé de flottation par mousse d'un minerai de phosphate selon l'une quelconque des revendications 1 à 12, le procédé comprenant :
facultativement, l'ajout d'un agent dépresseur au minerai ;
l'ajout du collecteur primaire et de l'auxiliaire pour le collecteur selon l'une quelconque des revendications 1 à 12 au minerai ;
facultativement, l'ajout d'un ou plusieurs composants supplémentaires au minerai sélectionnés dans le groupe des agents d'ajustement du pH, des dispersants et d'un collecteur secondaire ;
dans lequel le collecteur primaire, l'auxiliaire pour le collecteur et le collecteur secondaire facultatif peuvent être ajoutés les uns après les autres ou simultanément ;
le conditionnement du minerai en présence du collecteur primaire, du collecteur secondaire facultatif et de l'auxiliaire pour le collecteur ;
ensuite, facultativement l'ajout d'un ou plusieurs composants supplémentaires au minerai conditionné sélectionnés dans le groupe des agents d'ajustement du pH, des dispersants et des agents moussants ;
et
la mise en oeuvre d'un procédé de flottation par mousse pour récupérer les matériaux contenant du phosphate du minerai.

14. Procédé selon la revendication 13, dans lequel le collecteur secondaire est sélectionné dans le groupe des composés collecteurs anioniques, des composés collecteurs non ioniques ou de mélanges de deux de ceux-ci ou plus, dans lequel le composé collecteur anionique est sélectionné dans le groupe des acides gras, des sulfosuccinates d'alkyle, des maléates d'alkyle, des amidocarboxylates d'alkyle, des esters d'amidocarboxylates d'alkyle, des benzènesulfonates d'alkyle, des sulfonates d'alkyle et des acides gras sulfonés et le composé collecteur non ionique est sélectionné dans le groupe des éthoxylates, des glycosides et des éthanolamides, de préférence le composé collecteur non ionique est sélectionné dans le groupe des alcools en C11 à C24 éthoxylés ramifiés et non ramifiés, des alkylamines en C10 à C24 éthoxylées, des tensioactifs de sucre, des acides gras en C10 à C24 éthoxylés.

15. Procédé selon la revendication 13 ou 14, dans lequel l'agent moussant est sélectionné dans le groupe des huiles de pin, du MIBC (méthylisobutylcarbinal) et des alcools et des éthoxylates d'alcool, de préférence des alcools en C6 à C10 et des éthoxylates de ceux-ci.
